

# UNITED STATES PATENT OFFICE.

THOMAS ABRAHAM BAYLISS, OF WARWICK, ENGLAND, ASSIGNOR OF ONE-HALF TO  
BYRON GEORGE CLARK, OF LONDON, ENGLAND.

## ALLOY OF ZINC.

1,074,234.

Specification of Letters Patent. Patented Sept. 30, 1913.

No Drawing.

Application filed May 10, 1912. Serial No. 696,479.

To all whom it may concern:

Be it known that I, THOMAS ABRAHAM BAYLISS, a subject of the King of England, residing at Warwick, England, have invented certain new and useful Improvements in Alloys of Zinc, of which the following is a specification.

This invention relates to improvements in alloys of zinc containing zinc, aluminium and lead.

According to this invention an alloy of zinc, aluminium and lead, which shall be malleable, is produced in which the ingredients are present in the finished alloy in proportions between the limits of—

|           |              |
|-----------|--------------|
| Zinc      | 99.1 %—99.9% |
| Aluminium | 0.001%—0.9%  |
| Lead      | 0.01 %—0.0%  |

20 A preferred method of manufacturing the alloy according to the present invention is as follows:—The zinc and lead are melted in a pot or furnace closed to avoid oxidation. The temperature is raised to and 25 maintained between 350—450° C. to bring the zinc and lead into a molten condition and, while the zinc and lead are still in a molten condition, the aluminium is then added in a solid or molten state to make the 30 composition required. When the aluminium has become evenly disseminated throughout the mass and the several components are melted and intimately mixed together ready for pouring the metal is fluxed with ammonium chlorid or other suitable flux, skimmed and poured into molds to form slabs suitable for rolling. The alloy cools and sets in the mold and when a sufficiently low temperature has been reached (about 150—40 200° C.) the slabs are submitted to their first rolling. Sheets are thus made of convenient size according to requirements and subsequently annealed at a temperature of 200—250° C. in a furnace suitably arranged 45 and heated for that purpose. This annealing, which may be repeated as required, gives the requisite heat for subsequently rolling the sheets to the required dimensions and the final annealing operation follows 50 under similar conditions. The metal thus obtained is extremely tough and strong and is malleable and suitable for stamping and

like purposes, or for strip, wire and the like. It may be rolled into long lengths such as lengths of 100 ft. or 200 ft. or the like suitable for commercial requirements.

The metals may be present in any proportions within the limits set forth herein and in practice a good mixture is found to be obtained when the proportions are—

|           |        |
|-----------|--------|
| Zinc      | 99.85% |
| Aluminium | 0.1 %  |
| Lead      | 0.05%  |

What I claim as my invention and desire to secure by Letters Patent is:—

1. A malleable alloy composed of zinc, aluminium and lead in proportions between the limits of zinc 99.1%—99.9%; aluminium 0.001%—0.9%; and lead 0.01%—0.9%.

2. A malleable alloy containing 99.85% of zinc; 0.1% of aluminium; and 0.05% of lead.

3. A method of preparing a malleable alloy of zinc, aluminium and lead which consists in heating together zinc and lead to bring them into a molten condition while the zinc and lead are still in a molten condition, adding aluminium thereto to make the composition required, adding a flux thereto and allowing the alloy to cool and set, thereafter rolling it and subsequently annealing it.

4. A method of preparing a malleable alloy of zinc, aluminium and lead which consists in heating together zinc and lead to bring them into a molten condition, then while the zinc and lead are still in a molten condition adding aluminium thereto to make the composition required, maintaining the mixture in a molten condition until the aluminium has become evenly disseminated throughout the mass, adding a flux thereto and allowing the alloy to cool and set, thereafter rolling it and subsequently annealing it.

In testimony whereof I have signed my name to this specification in the presence of two subscribing witnesses.

THOMAS ABRAHAM BAYLISS.

Witnesses:

ALBERT ADAMS,  
ERNEST ALBERT JAMES.